

G. W. ELMEN.  
ELECTRODE.  
APPLICATION FILED AUG. 30, 1906.

Patented Mar. 25, 1913.

1,057,046

Fig. 1.



Fig. 2.



Witnesses:

Benjamin B. Hale  
Helen O'Neal

Inventor:  
Gustav W. Elmen  
by Alfred S. Davis  
His Attorney

# UNITED STATES PATENT OFFICE.

GUSTAV W. ELMEN, OF SCHENECTADY, NEW YORK, ASSIGNOR TO GENERAL ELECTRIC COMPANY, A CORPORATION OF NEW YORK.

## ELECTRODE.

1,057,046.

Specification of Letters Patent. Patented Mar. 25, 1913.

Application filed August 30, 1906. Serial No. 332,583.

*To all whom it may concern:*

Be it known that I, GUSTAV W. ELMEN, a subject of the King of Norway and Sweden, residing at Schenectady, county of Schenectady, State of New York, have invented certain new and useful Improvements in Electrodes, of which the following is a specification.

This invention relates to electrodes, and 10 more particularly to that general class of electrodes used for producing what are known as luminous or flaming arcs.

In general, my invention consists in adding to the material of the electrodes herein- 15 after specified a small quantity of a vaporizable compound for the purpose of steadyng the arc and preventing the flickerings and light variations which sometimes arise with electrodes of the flaming arc type.

20 I have found that sodium compounds are especially suited as arc-steadying ingredients, and although some sodium compounds appear to have a greater power than others, the following are typical of the general class 25 included in my invention:—sodium nitrate; sodium chlorate; sodium carbonate; sodium bichromate and sodium fluorid. Of these compounds, I consider sodium fluorid the most suitable, and I have found that even a 30 very small quantity of this material in the electrode effects wonderful results as a steadyng means.

The body of the electrode with which the sodium steadyng compound is associated 35 may consist of a variety of materials giving a luminous or flaming arc, but of this general class, electrodes consisting substantially of titanium compounds, such as the carbid or oxid, or of mixtures of titanium com- 40 pounds with iron compounds, are typical.

In order that my invention may be better understood I have hereinafter described it as applied to so-called magnetite electrodes containing magnetic oxid of iron, titanium 45 oxid and chromite. Such electrodes may be made by mixing and grinding together thirty parts of rutile, seventy parts of magnetite and twelve and one-half parts of chromite. It is to this mixture, or to similar 50 mixtures of which this one is typical, that I add a small quantity of a sodium compound to steady the arc when the electrode is in use.

55 Unsteadiness in the arc may result from one of several different causes, and although

I do not consider it necessary to explain in detail why the lamp is unsteady or why it flickers, I have hereinafter pointed out two sources of unsteadiness, and have explained how the sodium compound is used to overcome these undesirable features. 60

In the accompanying drawing, Figure 1 is a longitudinal section of an electrode embodying my invention, showing the upper end of the electrode as it appears after running a few hours in a lamp; Fig. 2 is an elevation of two electrodes showing the arc between them as produced in accordance with my invention.

Flaming arc electrodes may be of various 70 forms and sizes and may be manufactured in different ways, but the species shown in Fig. 1 is typical. It consists of a sheet iron envelop 1 having a metal closure 2 at the bottom, and containing a filling 3 of the 75 electrode material. When this filling is to consist of chromite, magnetite and rutile, in the proportions heretofore mentioned, I mix with it approximately one-quarter of one per cent. sodium fluorid, adding this material before the mixing and grinding operation, so that it may become intimately associated with the other components. This mixture may be moistened with water to render it somewhat plastic and may be 80 packed or tamped into the sheet iron tube 1. When the electrode is in use, this sheet iron envelop melts and wastes away with the filling so that the end of the electrode presents a smooth and somewhat rounded 85 surface. If the lamp is extinguished after several hours of operation, the hot material at the end of the electrode forms a smooth and dense cap over the end of the electrode. This cap is however sufficiently conductive 90 to permit re-lighting of the arc without difficulty. 95

When an electrode composed of the material above indicated, but without the addition of sodium fluorid, is operated, a pit or 100 crater is formed in the lower electrode, which becomes deeper and wider as the operation of the lamp continues; and in extreme cases the upper end of the electrode may become entirely hollowed out. After 105 the arc has been maintained for about 18 hours, the crater disappears and the end of the electrode assumes the general contour shown in Fig. 1; but during the time that the crater forms and persists, the apex of 110

the arc shifts about on the edge of the pit or crater and the light fluctuates in a very annoying manner.

In addition to the source of instability above mentioned, there is another source which I prefer to designate as "wandering" of the arc. I find that electrodes which do not contain the sodium compound yield an arc which meanders about over the electrode, 10 apparently seeking a new location for the cathode spot. This migration of the arc is so rapid that the arc appears to vibrate and tremble. I find that this shifting of the arc is also present when the electrode contains 15 sodium fluorid or other sodium compound, but for some reason, the rate of motion is greatly decreased and the arc moves so slowly over the electrode surface that there is no apparent flicker or other unsteadiness 20 in the light.

I have mentioned the use of sodium fluorid in the proportion of one-quarter of one per cent., and although I may depart somewhat from this proportion, I consider it advisable 25 to keep the quantity of sodium fluorid low. If too much is added the compound appears to cause a fusion or melting down of the end of the electrode in such a way that when the lamp is stopped, a substantially non-conducting button forms on the end of the electrode and the lamp will not again start until this button is removed. One-quarter of one per cent. of sodium fluorid does not change the color of the arc appreciably, although, 30 35 of course, the presence of sodium can be detected with a spectroscope. Another reason exists why the proportion of sodium compound should be kept low, and that is the peculiar lifting of the luminous cone of the 40 arc which takes place when the electrode contains an excess of the sodium compound. Fig. 4 represents diagrammatically a luminous arc running under normal conditions. From the upper electrode 7 depends a cone 45 shaped arc 8 the apex of which just touches the top of the negative electrode 9. This

cone is the source of a large amount of the light radiated by the arc, although the vapors which surround the cone are also luminous. In case the electrode contains an excess of the sodium compound, or in case compounds of other metals are substituted, there is a tendency for this luminous cone 8 to periodically lift or be forced away from the negative electrode 9. The lifting of the cone 50 is only momentary and produces nothing more serious than an instantaneous decrease in light intensity, but as this decrease may amount to as much as fifty per cent. of the entire light delivered by the arc, the phenomenon is objectionable. The immediate cause of this change in the luminous cone is obscure. With some electrodes the cone never lifts, with others it may lift only once a night, while with others it may lift every 55 60 65 five or six minutes throughout the entire life of the electrode. Whatever the cause of this instability may be, I find that a sodium compound such as sodium fluorid may safely be used with the electrode mixture in the 70 proportion of one-quarter of one per cent., without danger of causing any appreciable lifting of the arc cone, or in fact, any objectionable phenomena.

What I claim as new and desire to secure 75 by Letters Patent of the United States, is,—

1. A metallic flaming arc lamp electrode containing substantially one-quarter of one per cent. sodium fluorid.

2. An arc lamp electrode consisting of a 80 metal tube and a filling therefor composed of a mixture of iron oxid, rutile and chromite and about one-quarter of one per cent. of sodium fluorid.

3. An essentially metallic arc light pencil 85 comprising fluorid of an alkaline metal.

In witness whereof, I have hereunto set my hand this 25th day of August, 1906.

GUSTAV W. ELMEN.

Witnesses:

BENJAMIN B. HULL,  
HELEN ORFORD.